

## UNITED STATES PATENT OFFICE

2,391,842

## LUBRICATING GREASES

John D. Morgan, South Orange, N. J., assignor to  
 Cities Service Oil Company, New York, N. Y.,  
 a corporation of Pennsylvania

No Drawing. Application October 16, 1942,  
 Serial No. 462,221

12 Claims. (Cl. 252—37)

This invention relates to improvements in lubricants and more particularly to lubricating greases containing a liquid lubricating oil or medium and a silver soap.

I have discovered that silver soaps, for example, the soaps made from soap-forming fatty materials such as the higher fatty acids, give lubricants of unusual properties which are quite different from those made from the usual alkali and alkaline earth metal soaps.

One of the serious problems of the present time is the provision of suitable greases for use at low temperatures. The ordinary greases made from mineral lubricating oils and sodium, calcium, aluminum, and other soaps, become hard and stiff and fail to lubricate at low temperatures, sometimes even at temperatures as low as zero degrees F. Greases containing silver soap have been found to be stable and plastic over relatively wide temperature ranges, and to be especially adaptable for lubricating various bearings of aircraft in which a grease must be used instead of a liquid lubricant.

The features of the present invention may be illustrated by reference to the following examples of lubricant compositions containing silver soaps, in which the quantities of the various ingredients are given in parts by weight.

*Example No. 1*

A grease found to be useful at extremely low temperatures of the order of about minus 70° F., was prepared by heating a mixture of about 86 parts of a Ponca City lubricating oil stock, having a Saybolt Universal viscosity at 100° F. of 72.5 seconds, and about 7.5 parts of silver stearate, to a temperature of 400° F. The mixture was heated gradually up to this temperature, and it was noted that at a temperature of about 220° F. the mixture began to turn to a blue-black color. The final mixture was cooled quickly in thin layers. A fine, soft gel was produced.

This grease passed the Navy test for low temperature greases which is conducted with a ball-bearing tester at a temperature of minus 67° F. The Navy limit for low temperature grease is thirty seconds for one revolution on this tester, whereas the time recorded for the grease described above was 20 seconds.

The silver stearate used in making the above grease was prepared by first making potassium stearate from KOH and stearic acid, and then reacting the potassium stearate with silver nitrate. The resulting reaction mixture was filtered, the precipitate washed to remove any po-

tassium nitrate, and finally dried in an oven at 220° F. The silver soaps are practically insoluble in water, and are preferably dispersed in liquid organic lubricants in a substantially dry state.

*Example No. 2*

10 A slightly heavier grease was prepared by the procedure followed in Example No. 1, by heating a mixture of 87.6 parts of the same mineral lubricating oil stock, 11.2 parts of silver stearate, and 1.4 parts of aluminum stearate. This grease also passed the Navy test for a low temperature grease and was found to have high load-carrying characteristics. In a test carried out on a 4-ball testing machine, there was no seizure up to and including a gage pressure of 1000 lbs., and only an eight division friction rise over the whole pressure range. This result is to be compared with a gage load of about 250 lbs, which is registered on the 4-ball machine at the point of seizure in the case of a light Spindle oil.

*Example No. 3*

25 A slightly modified grease from that of Example No. 1 was prepared from the same lubricating oil stock and silver stearate, by including in the mixture during the heating operation a small proportion of a rubber latex. This mixture comprised about 85 parts of the mineral lubricating oil, about 8 parts of silver stearate, and about one part of rubber latex. The properties of this grease was similar to that of Example No. 1 but it was found to be more adherent.

30 Light, medium or heavy greases may be made for particular purposes by varying the viscosity of the liquid lubricating oil, the quantity of silver soap, and the quantities of other constituents which may be added to the compositions. The term "liquid lubricant" or "lubricating oil" as used in connection with this invention, is not restricted to mineral lubricating oils, but is to be understood to include other liquid lubricants, such as vegetable and animal base oils, as well as commercial or pure compounds which have lubricating properties. Examples of such compounds are: trichlorobenzene, butyl oxalate, methyl benzoate, butyl benzoate, butyl acetyl ricinoleate, amyl stearate, diethyl and dibutyl phthalates, diethyl naphthalene, tributyl and tricresyl phosphates, decalin, tetralin, normal hexyl ether, and halowax oils. Many of these liquid lubricants have been found to be unusually effective, even when used alone at low temperatures, and their use is therefore especially effective in making low temperature greases with silver soaps.

While the invention has been illustrated in connection with the use of silver stearate, other silver soaps of fats or fatty acids may be used, such as silver laurate, silver oleate, silver palmitate, silver resinate, and silver soaps of whale oil, castor oil, etc. Most of these soaps have melting points in the neighborhood of about 200° C. In making greases in accordance with the present invention the proportion of silver soap may be varied from 4% to 20% of the composition, and the composition may, if desired, include from 1% to 3% of an aluminum soap of one of the fatty materials mentioned above, such as aluminum stearate, and where rubber latex or equivalent elastic polymer is used in the grease, it may comprise from 1% to 2% of the composition. Instead of using rubber latex, synthetic rubbers may be used, or balata, chlorinated rubber, gum rubber, butyl rubber and others. The addition of small proportions of silver soap to a lubricating liquid or oil increases its load-carrying properties, prevents leakage from bearings, and improves the lubricating properties of the liquid or oil.

Any of the greases made in accordance with the present invention may include a small proportion of an antioxidant or anticorrosion agent which may be found necessary or advisable in the case of any particular liquid lubricating medium or particular bearing metals involved. Tributyl, triphenyl, and tricresyl phosphites may be used as well as other known anticorrosion and antioxidantizing agents.

It is to be understood that although the features of the invention have been described and illustrated in connection with certain specific examples, the invention, however, is not to be limited thereto or otherwise restricted, except by the prior art and the scope of the appended claims.

Having described the invention and illustrated the same in connection with certain specific examples, what is claimed as new is:

1. A lubricating composition having a grease structure made by heating a mixture comprised principally of a lubricating oil and from about 4% to about 20% by weight of a silver soap of a higher fatty acid to a temperature of approximately 400° F., said composition having a stable plastic gel-like consistency.

2. A lubricating grease composition comprised principally of approximately 92 per cent by weight of a mineral lubricating oil and approximately 8 per cent by weight of silver stearate, said composition having a stable plastic gel-like consistency resulting from the heating of a mixture of said ingredients to a temperature of approximately 400° F. followed by cooling.

3. A lubricating grease composition comprised principally of a liquid lubricating medium, from approximately 4 to approximately 20 per cent by weight of a silver soap of soap-forming fatty material, and from one to three per cent by weight of aluminum soap of a soap-forming fatty material, said composition having a stable plas-

tic gel-like consistency resulting from the heating of a mixture of said ingredients to a temperature of approximately 400° F. followed by cooling.

4. A lubricating grease composition having a plastic gel-like consistency made by heating a mixture of a liquid oily lubricant, a silver soap and an aluminum soap to a temperature of approximately 400° F., said silver soap being the major grease-forming agent and being present in the composition in sufficient proportion to substantially thicken the liquid oily lubricant.

5. A lubricating grease composition having a plastic gel-like consistency and containing a major proportion of a liquid lubricating oil, a substantial proportion of a silver soap of a soap-forming fatty material serving as the major grease forming ingredient, a small proportion of an aluminum soap and a small proportion of an elastic polymer, said composition being formed by heating a mixture of said ingredient to a temperature of approximately 400° F. followed by subsequent cooling.

6. The method of making a silver soap grease comprising heating a mixture comprised mostly of a liquid lubricating medium and from approximately 4% to approximately 20% by weight of a silver soap of a soap-forming fatty material to a temperature of approximately 400° F., effecting the heating operation gradually to the final temperature and thereafter quickly cooling the mixture in thin layers to produce a stable plastic grease.

7. The method of making a silver soap grease as defined by claim 6 in which the initial mixture includes from about 1% to about 3% of an aluminum soap of a soap-forming fatty material.

8. The method of making a silver soap grease as defined by claim 6 in which the initial mixture includes a small proportion of an elastic polymer sufficient to increase the adherent properties of the resulting grease.

9. The method of making silver soap grease as defined by claim 6 in which a substantially dry silver soap is employed.

10. A lubricating grease composition in accordance with claim 3 in which said silver soap is silver stearate.

11. A lubricating grease composition in accordance with claim 3 in which said silver soap is silver stearate, and said aluminum soap is aluminum stearate.

12. A lubricating grease composition consisting essentially of approximately 87.5 per cent by weight of a mineral lubricating oil, about 11 per cent by weight of silver stearate, and about 1½ per cent by weight of aluminum stearate, said composition having a stable plastic gel-like consistency resulting from the heating of the mixture of said ingredients to a temperature of approximately 400° F. followed by cooling.

JOHN D. MORGAN.